

# United States Patent

Bindler

[15] 3,652,201

[45] Mar. 28, 1972

[54] **PROCESS FOR THE PRODUCTION OF DYEINGS ON FIBER MATERIAL CONSISTING OF POLYMERIC OR COPOLYMERIC ACRYLONITRILE**

[72] Inventor: **Jakob Bindler**, Riehen, Switzerland

[73] Assignee: **Ciba-Geigy AG**, Basel, Switzerland

[22] Filed: **Apr. 28, 1969**

[21] Appl. No.: **819,976**

[30] **Foreign Application Priority Data**

Apr. 30, 1968 Switzerland ..... 6438/68

[52] U.S. Cl. .... 8/172, 8/177 AB

[51] Int. Cl. .... D06p 5/06

[58] Field of Search ..... 8/172, 84, 177 AB

[56] **References Cited**

UNITED STATES PATENTS

2,986,444 5/1961 Rokohl et al. .... 8/177 AB  
2,989,361 6/1961 Hees ..... 8/84 X  
3,104,933 9/1963 Mendelsohn et al. .... 8/172 X

Primary Examiner—George F. Lesmes  
Assistant Examiner—T. J. Herbert, Jr.  
Attorney—Wenderoth, Lind & Ponack

[57]

## ABSTRACT

A process for the production of level dyeings on polymeric or copolymeric acrylonitrile fibers by dyeing said fibers with a dye liquor containing a basic dyestuff and as dye assistant a quaternary ammonium compound of the formula



wherein

$\text{R}_1$  represents an aliphatic hydrocarbon radical with at least eight carbon atoms,

$\text{R}_2$  represents a lower alkyl radical,

$\text{R}_3$  represents a lower alkyl radical optionally substituted by hydroxyl and/or phenyl groups,

$\text{R}_4$  represents a lower alkylene bridge and

$\text{X}^-$  represents the anion equivalent of an acid usch as, e.g.,  $\text{Cl}^-$  or  $\text{Br}^-$  is, described.

The dyeing process is distinguished from those using known strong cationic retarders by its adequate retarding action without any undue blocking effect.

**9 Claims, No Drawings**

PROCESS FOR THE PRODUCTION OF DYEINGS ON  
FIBER MATERIAL CONSISTING OF POLYMERIC OR  
COPOLYMERIC ACRYLONITRILE

The present invention concerns a process for the production of even dyeings on fiber material consisting of polymeric or copolymeric acrylonitrile, the dye liquor applicable for the process and the material evenly dyed therewith.

Hitherto, in order to dye polymeric or copolymeric acrylonitrile by the exhaustion method with basic dyestuffs and in level shades, a dye liquor has been used which, in addition to basic dyestuffs, contained as dye assistants tertiary, mono- or bis-quaternary organic nitrogen compounds having at least one higher alkyl radical per molecule. As a rule, these assistants detrimentally affect the fastness to light of the dyeings obtained and "block" the fibers, i.e., as soon as a portion thereof has been drawn onto the fiber, they reduce the absorption power of the fiber both for further basic dyestuff and for further dye assistant.

This blocking effect on the fiber makes the re-dyeing and in particular the cross dyeing of a shade already attained very much more difficult. Since the blocking effect caused by the known dye assistants on the polyacrylonitrile fiber affects the individual basic dyestuffs present, for instance, in a conventional mixed dye in different degrees, it is also generally impossible to attain or reproduce a desired shade with usually preferred mixtures of basic dyestuffs. Finally the blocking effect has a varying influence on the rate at which the basic dyestuffs draw onto the aforesaid type of fibers which, in practice, easily leads to uneven distribution of the dyestuff. Moreover, since the hitherto used dye assistants which have drawn onto the fiber are very difficult to remove, this blocking effect is generally irreversible.

In contrast thereto, the claimed quaternary organic nitrogen compounds, in addition to exhibiting the said "blocking effect," are also effective "retarders," that is they exert a reversible restraining effect upon the rate at which the basic dyestuff in the bath dyes the fiber. Consequently, the use of such retarders leads to uniform dyeings from a bath which is virtually exhausted at the end of the dyeing operation.

It has been found that fiber material consisting of polymeric or copolymeric acrylonitrile can be dyed in even shades if this material is dyed using an acid dye liquor, preferably acetic acid dye liquor, which contains at least one cationic dyestuff and a quaternary ammonium compound of the formula



wherein

$\text{R}_1$  represents an aliphatic hydrocarbon radical with at least eight carbon atoms,

$\text{R}_2$  represents a lower alkyl radical,

$\text{R}_3$  represents an lower alkyl radical optionally substituted by hydroxyl and/or phenyl groups,

$\text{R}_4$  represents a lower alkylene bridge and

$\text{X}^-$  represents the anion equivalent of an acid such as, e.g.,  $\text{Cl}^-$  or  $\text{Br}^-$ .

The aliphatic hydrocarbon radical  $\text{R}_1$  can be saturated or unsaturated, straight or branched. It has at least eight and preferably 12 to 14 carbon atoms. Examples for  $\text{R}_1$  are the octyl, decyl, dodecyl or myristyl radical.

The lower alkyl radicals  $\text{R}_2$  and  $\text{R}_3$  — when the latter represents an lower alkyl group — preferably have one to four carbon atoms and, in particular, they represent the methyl or ethyl radical. If  $\text{R}_3$  contains hydroxyl and/or phenyl groups, then these are preferably in the terminal ( $\omega$ -)position. Such substituted lower alkyl radicals are, e.g., the  $\beta$ -hydroxyethyl,  $\gamma$ -hydroxypropyl and  $\beta$ -hydroxy- $\beta$ -phenylethyl group.

The alkylene bridge  $\text{R}_4$  preferably has at most three carbon atoms and represents especially the methylene group.

In this specification including the claims the term "lower" is used to denote an alkyl radical having at most five carbon atoms.

The quaternary ammonium compounds, applicable according to the invention, are accessible in various ways, e.g., by reacting 1,3-dichloro-propanol-2, 1,4-dichloro-butanol-3, 1,5-dichloro-pentanol-4 or preferably epihalogen hydrins, such as epibromohydrin or especially epichlorohydrin, with tertiary amines such as N,N-dimethyl-N-octylamine, N,N-diethyl-N-octylamine, N,N-dimethyl-N-dodecylamine, N,N-diethyl-N-dodecylamine, N-methyl-N-isopropyl-N-dodecylamine, N-methyl-N-benzyl-N-dodecylamine, N-methyl-N- $\beta$ -phenylethyl-N-dodecylamine, N,N-dimethyl-N-myristylamine or with tertiary amines which have been produced by addition of equivalent amounts of alkylene oxide or styrene oxide to a fatty amine having an aliphatic hydrocarbon radical and a lower alkyl radical such as, e.g., N-methyl-N-octylamine, N-methyl-N-dodecylamine, N-ethyl-N-dodecylamine, N-isopropyl-N-dodecylamine, N-propyl-N-dodecylamine, N-butyl-N-dodecylamine or N-methyl-N-myristylamine. The reaction of the tertiary amines with e.g., epihalogen hydrins to give the quaternary ammonium compounds is performed by heating the components to temperatures between 50° and 100° C., optionally in organic solvents, preferably in the presence of aluminum chloride, tin tetrachloride or boron trifluoride. Suitable organic solvents are, optionally, halogenated aromatic hydrocarbons, e.g., benzene, toluene or xylols, chlorobenzene, dichlorobenzene or trichlorobenzene as well as, optionally, halogenated aliphatic hydrocarbons such as carbon tetrachloride, trichloroethylene or methylene chloride.

Of particular value as levelling agents are the quaternary ammonium salts, applicable according to the invention, wherein  $\text{R}_1$  represents an alkyl radical with eight to 14 carbon atoms,  $\text{R}_2$  and  $\text{R}_3$  each represent the methyl or ethyl group,  $\text{R}_4$  the methylene bridge and  $\text{X}^-$  the chlorine or bromine ion.

An excellent levelling action without the formation of froth is exhibited by quaternary ammonium salts, applicable according to the invention, which are derived from styrene oxide, especially N-methyl-N-dodecyl-N- $\beta$ -hydroxy- $\beta$ -phenylethyl-N-2,3-epoxypropyl ammonium chloride.

Suitable as cationic dyestuffs applicable according to the invention are, advantageously, the technically easily accessible salts and metal halides, e.g., zinc chloride double salts of the known basic dyestuffs. These are, e.g., thiazines, oxazines, diphenyl methane, triphenyl methane, rhodamines, azo- or anthra-quinone dyestuffs and preferably monoazo, methine and azomethine dyestuffs, all containing onium groups, whereby as onium groups reference is made, above all, to ammonium groups.

As fiber material consisting of polymeric and copolymeric acrylonitrile, such fiber materials are suitable, the fiber-forming substance of which consists of a synthetic, longchained polymer containing at least 85 acrylonitrile. In the case of the acid groups of copolymeric producing the dyestuff affinity, suitable groups are primarily carboxylic acid groups, carboxylic acid amide groups or hydroxyl groups, and also sulphonate groups.

The polyacrylonitrile fibers can be dyed, according to the invention, in any desired form, e.g., as loose material or in the form of slubbing, yarn, hank or on cheeses or as fabrics. They can also be dyed according to the invention in admixture with other fibers, e.g., with cellulose or polyamide fibers, especially however with wool.

The dyeing of the fiber material is performed using the exhaust process from short, concentrated dyebaths (goods/liquor ratio 1:5), and also from long dyebaths (goods/liquor ratio 1:100 at temperatures of preferably 60° to 100° C.). The finished fiber material is finally rinsed and dried.

Depending on the desired depth of color, the contents of quaternary ammonium salt, according to the invention, in the dye bath is between 0.02 and 0.5 g. per liter of liquor. Less levelling agent is required for deep dyeings than for light shades.

The acid reaction of the liquor is adjusted preferably using organic acid, especially acetic acid. For example, 40% acetic acid is added in quantities of 0.5 to 5 ml. per liter of liquor. In addition, in order to ensure pH values of the liquor of preferably from 3.5 to 5, small amounts of sulphuric acid and/or neutral salts, such as sodium sulphate or sodium chloride, are added to the dye bath.

The dyeings obtained according to the invention on polymeric and copolymeric acrylonitrile fibers are characterized by a very good uniformity. Of particular advantage is the fact that the quaternary ammonium salts applicable according to the invention, compared with known cationic retarding agents of similar constitution, also have, in addition to an adequate retarding action, a lower blocking action. They are therefore very suitable for correcting faulty dyeings and for cross-dyeing, without impairing the dyestuff yield and the fastness properties of the obtained dyeings.

The following Examples illustrate the invention, whereby the temperature are given in degrees Centigrade C.I. denotes COLOR INDEX, Second Edition, 1956, published by The Society of Dyers and Colourists, Bradford, England and The American Association of Textile Chemists and Colorists, Lowell, Mass. USA.

#### EXAMPLE 1

25 g. of polyacrylonitrile yarn are introduced at 50° into a liter of dye liquor containing 0.12 g. of the cationic dyestuff of the formula



0.05 g. of N,N-dimethyl-N-dodecyl-N-2,3-epoxypropyl ammonium chloride and 0.5 ml. of 40% acetic acid. The temperature of the dye bath is raised to boiling point and the dye bath is held at this temperature for 1 hour. After cooling to 60°, the dyed material is taken out and it is then rinsed with lukewarm and cold water.

A red dyed yarn is obtained of excellent uniformity.

The N,N-dimethyl-N-dodecyl-N-2,3-epoxypropyl ammonium chloride used in the first section can, for example, be produced as follows:

68 g. of N,N-dimethyl-N-dodecylamine together with 0.1 g. of aluminum chloride are heated to 98°-100°. 30 g. of epichlorohydrin are then added dropwise within 30 minutes. After stirring for 3 hours at 100°-105°, a thick brown paste is obtained, which dissolves in water in a practically clear form.

#### EXAMPLE 2

25 g. of polyacrylonitrile fabric are introduced at 50° into a liter of dye liquor containing 0.075 g. of the cationic dyestuff of the formula



5 0.125 g. of N,N-dimethyl-N-dodecyl-N-2,3-epoxypropyl ammonium chloride, 0.040 ml. of 98% sulphuric acid, 1.5 ml. of 40% acetic acid and 2.5 g. of anhydrous sodium sulphate. The temperature of the dye bath is raised to the boiling point and dyeing proceeds at this temperature for 1 hour. The thus dyed material is then taken out and rinsed with lukewarm and cold water. A very uniform, blue dyeing on polyacrylonitrile fabric is obtained.

10 If, instead of 0.125 g. of N,N-dimethyl-N-dodecyl-N-2,3-epoxypropyl ammonium chloride, the same amounts are used of N,N-diethyl-N-dodecyl-N-2,3-epoxypropyl ammonium chloride, N-methyl-N-β-hydroxy-ethyl-N-dodecyl-N-2,3-epoxypropyl ammonium chloride or N-methyl-N-β-hydroxypropyl-N-dodecyl-N-2,3-epoxypropyl ammonium chloride, 15 using otherwise the procedure given in the example, dyeings of good uniformity are obtained.

#### EXAMPLE 3

20 25 g. of polyacrylonitrile yarn are introduced at 50° into a liter of dye liquor 85% 0.2 g. of the cationic dyestuff of the formula



25 30 0.125 g. of N-dodecyl-N-methyl-N-2,3-epoxypropyl-N-β-hydroxy-β-phenylethyl ammonium chloride and 0.5 ml. of 40% acetic acid. The temperature of the dye bath is raised to the boiling point and the dye bath is held at this temperature for 1 hour. After cooling to 60°, the dyed material is taken out and then rinsed with lukewarm and cold water.

35 A very uniformly red dyed polyacrylonitrile yarn is obtained.

The N-dodecyl-N-methyl-N-2,3-epoxypropyl-N-β-hydroxy-β-phenylethyl ammonium chloride used in the first section can, for example, be produced as follows: 37 g. of styrene oxide are added dropwise at 45°-50°, while stirring, to a solution of 60 g. of N-methyl-N-dodecylamine in 300 g. of chlorobenzene. The reaction mixture is heated to boiling and is refluxed for 10 hours at boiling temperature. The chlorobenzene is then distilled off in vacuo and the residue is distilled under reduced pressure at B.P. 153°-155°.

40 45 50 55 60 65 70 75 76 77 78 79 80 81 82 83 84 85 86 87 88 89 90 91 92 93 94 95 96 97 98 99 100 101 102 103 104 105 106 107 108 109 110 111 112 113 114 115 116 117 118 119 120 121 122 123 124 125 126 127 128 129 130 131 132 133 134 135 136 137 138 139 140 141 142 143 144 145 146 147 148 149 150 151 152 153 154 155 156 157 158 159 160 161 162 163 164 165 166 167 168 169 170 171 172 173 174 175 176 177 178 179 180 181 182 183 184 185 186 187 188 189 190 191 192 193 194 195 196 197 198 199 200 201 202 203 204 205 206 207 208 209 210 211 212 213 214 215 216 217 218 219 220 221 222 223 224 225 226 227 228 229 230 231 232 233 234 235 236 237 238 239 240 241 242 243 244 245 246 247 248 249 250 251 252 253 254 255 256 257 258 259 260 261 262 263 264 265 266 267 268 269 270 271 272 273 274 275 276 277 278 279 280 281 282 283 284 285 286 287 288 289 290 291 292 293 294 295 296 297 298 299 300 301 302 303 304 305 306 307 308 309 310 311 312 313 314 315 316 317 318 319 320 321 322 323 324 325 326 327 328 329 330 331 332 333 334 335 336 337 338 339 340 341 342 343 344 345 346 347 348 349 350 351 352 353 354 355 356 357 358 359 360 361 362 363 364 365 366 367 368 369 370 371 372 373 374 375 376 377 378 379 380 381 382 383 384 385 386 387 388 389 390 391 392 393 394 395 396 397 398 399 400 401 402 403 404 405 406 407 408 409 410 411 412 413 414 415 416 417 418 419 420 421 422 423 424 425 426 427 428 429 430 431 432 433 434 435 436 437 438 439 440 441 442 443 444 445 446 447 448 449 450 451 452 453 454 455 456 457 458 459 460 461 462 463 464 465 466 467 468 469 470 471 472 473 474 475 476 477 478 479 480 481 482 483 484 485 486 487 488 489 490 491 492 493 494 495 496 497 498 499 500 501 502 503 504 505 506 507 508 509 510 511 512 513 514 515 516 517 518 519 520 521 522 523 524 525 526 527 528 529 530 531 532 533 534 535 536 537 538 539 540 541 542 543 544 545 546 547 548 549 550 551 552 553 554 555 556 557 558 559 560 561 562 563 564 565 566 567 568 569 570 571 572 573 574 575 576 577 578 579 580 581 582 583 584 585 586 587 588 589 5810 5811 5812 5813 5814 5815 5816 5817 5818 5819 5820 5821 5822 5823 5824 5825 5826 5827 5828 5829 5830 5831 5832 5833 5834 5835 5836 5837 5838 5839 5840 5841 5842 5843 5844 5845 5846 5847 5848 5849 5850 5851 5852 5853 5854 5855 5856 5857 5858 5859 5860 5861 5862 5863 5864 5865 5866 5867 5868 5869 5870 5871 5872 5873 5874 5875 5876 5877 5878 5879 5880 5881 5882 5883 5884 5885 5886 5887 5888 5889 5890 5891 5892 5893 5894 5895 5896 5897 5898 5899 58100 58101 58102 58103 58104 58105 58106 58107 58108 58109 58110 58111 58112 58113 58114 58115 58116 58117 58118 58119 58120 58121 58122 58123 58124 58125 58126 58127 58128 58129 58130 58131 58132 58133 58134 58135 58136 58137 58138 58139 58140 58141 58142 58143 58144 58145 58146 58147 58148 58149 58150 58151 58152 58153 58154 58155 58156 58157 58158 58159 58160 58161 58162 58163 58164 58165 58166 58167 58168 58169 58170 58171 58172 58173 58174 58175 58176 58177 58178 58179 58180 58181 58182 58183 58184 58185 58186 58187 58188 58189 58190 58191 58192 58193 58194 58195 58196 58197 58198 58199 58100 58101 58102 58103 58104 58105 58106 58107 58108 58109 58110 58111 58112 58113 58114 58115 58116 58117 58118 58119 58120 58121 58122 58123 58124 58125 58126 58127 58128 58129 58130 58131 58132 58133 58134 58135 58136 58137 58138 58139 58140 58141 58142 58143 58144 58145 58146 58147 58148 58149 58150 58151 58152 58153 58154 58155 58156 58157 58158 58159 58160 58161 58162 58163 58164 58165 58166 58167 58168 58169 58170 58171 58172 58173 58174 58175 58176 58177 58178 58179 58180 58181 58182 58183 58184 58185 58186 58187 58188 58189 58190 58191 58192 58193 58194 58195 58196 58197 58198 58199 58100 58101 58102 58103 58104 58105 58106 58107 58108 58109 58110 58111 58112 58113 58114 58115 58116 58117 58118 58119 58120 58121 58122 58123 58124 58125 58126 58127 58128 58129 58130 58131 58132 58133 58134 58135 58136 58137 58138 58139 58140 58141 58142 58143 58144 58145 58146 58147 58148 58149 58150 58151 58152 58153 58154 58155 58156 58157 58158 58159 58160 58161 58162 58163 58164 58165 58166 58167 58168 58169 58170 58171 58172 58173 58174 58175 58176 58177 58178 58179 58180 58181 58182 58183 58184 58185 58186 58187 58188 58189 58190 58191 58192 58193 58194 58195 58196 58197 58198 58199 58100 58101 58102 58103 58104 58105 58106 58107 58108 58109 58110 58111 58112 58113 58114 58115 58116 58117 58118 58119 58120 58121 58122 58123 58124 58125 58126 58127 58128 58129 58130 58131 58132 58133 58134 58135 58136 58137 58138 58139 58140 58141 58142 58143 58144 58145 58146 58147 58148 58149 58150 58151 58152 58153 58154 58155 58156 58157 58158 58159 58160 58161 58162 58163 58164 58165 58166 58167 58168 58169 58170 58171 58172 58173 58174 58175 58176 58177 58178 58179 58180 58181 58182 58183 58184 58185 58186 58187 58188 58189 58190 58191 58192 58193 58194 58195 58196 58197 58198 58199 58100 58101 58102 58103 58104 58105 58106 58107 58108 58109 58110 58111 58112 58113 58114 58115 58116 58117 58118 58119 58120 58121 58122 58123 58124 58125 58126 58127 58128 58129 58130 58131 58132 58133 58134 58135 58136 58137 58138 58139 58140 58141 58142 58143 58144 58145 58146 58147 58148 58149 58150 58151 58152 58153 58154 58155 58156 58157 58158 58159 58160 58161 58162 58163 58164 58165 58166 58167 58168 58169 58170 58171 58172 58173 58174 58175 58176 58177 58178 58179 58180 58181 58182 58183 58184 58185 58186 58187 58188 58189 58190 58191 58192 58193 58194 58195 58196 58197 58198 58199 58100 58101 58102 58103 58104 58105 58106 58107 58108 58109 58110 58111 58112 58113 58114 58115 58116 58117 58118 58119 58120 58121 58122 58123 58124 58125 58126 58127 58128 58129 58130 58131 58132 58133 58134 58135 58136 58137 58138 58139 58140 58141 58142 58143 58144 58145 58146 58147 58148 58149 58150 58151 58152 58153 58154 58155 58156 58157 58158 58159 58160 58161 58162 58163 58164 58165 58166 58167 58168 58169 58170 58171 58172 58173 58174 58175 58176 58177 58178 58179 58180 58181 58182 58183 58184 58185 58186 58187 58188 58189 58190 58191 58192 58193 58194 58195 58196 58197 58198 58199 58100 58101 58102 58103 58104 58105 58106 58107 58108 58109 58110 58111 58112 58113 58114 58115 58116 58117 58118 58119 58120 58121 58122 58123 58124 58125 58126 58127 58128 58129 58130 58131 58132 58133 58134 58135 58136 58137 58138 58139 58140 58141 58142 58143 58144 58145 58146 58147 58148 58149 58150 58151 58152 58153 58154 58155 58156 58157 58158 58159 58160 58161 58162 58163 58164 58165 58166 58167 58168 58169 58170 58171 58172 58173 58174 58175 58176 58177 58178 58179 58180 58181 58182 58183 58184 58185 58186 58187 58188 58189 58190 58191 58192 58193 58194 58195 58196 58197 58198 58199 58100 58101 58102 58103 58104 58105 58106 58107 58108 58109 58110 58111 58112 58113 58114 58115 58116 58117 58118 58119 58120 58121 58122 58123 58124 58125 58126 58127 58128 58129 58130 58131 58132 58133 58134 58135 58136 58137 58138 58139 58140 58141 58142 58143 58144 58145 58146 58147 58148 58149 58150 58151 58152 58153 58154 58155 58156 58157 58158 58159 58160 58161 58162 58163 58164 58165 58166 58167 58168 58169 58170 58171 58172 58173 58174 58175 58176 58177 58178 58179 58180 58181 58182 58183 58184 58185 58186 58187 58188 58189 58190 58191 58192 58193 58194 58195 58196 58197 58198 58199 58100 58101 58102 58103 58104 58105 58106 58107 58108 58109 58110 58111 58112 58113 58114 58115 58116 58117 58118 58119 58120 58121 58122 58123 58124 58125 58126 58127 58128 58129 58130 58131 58132 58133 58134 58135 58136 58137 58138 58139 58140 58141 58142 58143 58144 58145 58146 58147 58148 58149 58150 58151 58152 58153 58154 58155 58156 58157 58158 58159 58160 58161 58162 58163 58164 58165 58166 58167 58168 58169 58170 58171 58172 58173 58174 58175 58176 58177 58178 58179 58180 58181 58182 58183 58184 58185 58186 58187 58188 58189 58190 58191 58192 58193 58194 58195 58196 58197 58198 58199 58100 58101 58102 58103 58104 58105 58106 58107 58108 58109 58110 58111 58112 58113 58114 58115 58116 58117 58118 58119 58120 58121 58122 58123 58124 58125 58126 58127 58128 58129 58130 58131 58132 58133 58134 58135 58136 58137 58138 58139 58140 58141 58142 58143 58144 58145 58146 58147 58148 58149 58150 58151 58152 58153 58154 58155 58156 58157 58158 58159 58160 58161 58162 58163 58164 58165 58166 58167 58168 58169 58170 58171 58172 58173 58174 58175 58176 58177 58178 58179 58180 58181 58182 58183 58184 58185 58186 58187 58188 58189 58190 58191 58192 58193 58194 58195 58196 58197 58198 58199 58100 58101 58102 58103 58104 58105 58106 58107 58108 58109 58110 58111 58112 58113 58114 58115 58116 58117 58118 58119 58120 58121 58122 58123 58124 58125 58126 58127 58128 58129 58130 58131 58132 58133 58134 58135 58136 58137 58138 58139 58140 58141 58142 58143 58144 58145 58146 58147 58148 58149 58150 58151 58152 58153 58154 58155 58156 58157 58158 58159 58160 58161 58162 58163 58164 58165 58166 58167 58168 58169 58170 58171 58172 5

Table I—Continued

| G. amounts<br>of the<br>quaternary<br>ammonium<br>salts | Tertiary amine of the formula |                 |                               | Boiling point of the<br>tertiary amine in °C.                                             |                      |
|---------------------------------------------------------|-------------------------------|-----------------|-------------------------------|-------------------------------------------------------------------------------------------|----------------------|
|                                                         | $R_1$                         | $R_2$           | $R_3$                         |                                                                                           |                      |
| <b>Example No.:</b>                                     |                               |                 |                               |                                                                                           |                      |
| 6.....                                                  | 0.06                          | $-C_{12}H_{25}$ | $-C_2H_5$                     | do                                                                                        | B.P. 0.15mm. 160-161 |
| 7.....                                                  | 0.08                          | $-C_{12}H_{25}$ | $-CH-CH_3$<br>CH <sub>3</sub> | do                                                                                        | B.P. 0.1mm. 163-166  |
| 8.....                                                  | 0.06                          | $-C_{12}H_{25}$ | $-CH_2CH_2CH_3$               | do                                                                                        | B.P. 0.7mm. 160-162  |
| 9.....                                                  | 0.06                          | $-C_{12}H_{25}$ | $-C_4H_9$                     | do                                                                                        | B.P. 0.2mm. 166-169  |
| 10.....                                                 | 0.05                          | $-C_{12}H_{25}$ | $-CH_3$                       | $-CH_2$  | B.P. 0.01mm. 135-140 |

If, instead of 0.2 g. of the dyestuff given in example 3, corresponding amounts of the dyestuffs listed in table II, column II, are used, applying otherwise the same procedure, then dye-

ings are obtained in the shades given in column III having similar properties.

20

TABLE II

| I.      | II.                                                                                  | III.                                     |
|---------|--------------------------------------------------------------------------------------|------------------------------------------|
| Nr.     | Dyestuff                                                                             | Shade on<br>polycrylic<br>nitrile fibres |
| 11..... |    | Blue.                                    |
| 12..... |   | Red.                                     |
| 13..... |   | Yellow.                                  |
| 14..... |  | Do.                                      |
| 15..... |  | Blue.                                    |
| 16..... |  | Do.                                      |

TABLE II

| I.      | II.      | III.                                      |
|---------|----------|-------------------------------------------|
| Nr.     | Dyestuff | Shade on<br>polyacrylo-<br>nitrile fibres |
| 17..... |          | Orange.                                   |
| 18..... |          | Do.                                       |
| 19..... |          | Red.                                      |
| 20..... |          | Red.                                      |
| 21..... |          | Violet.                                   |
| 22..... |          | Do.                                       |
| 23..... |          | Reddish<br>yellow.                        |

TABLE II

| I.  | II.      | III.                                      |
|-----|----------|-------------------------------------------|
| Nr. | Dyestuff | Shade on<br>polyacrylo-<br>nitrile fibres |
| 24  |          | Red.                                      |
| 25  |          | Blue.                                     |
| 26  |          | Red.                                      |
| 27  |          | Red.                                      |
| 28  |          | Violet.                                   |
| 29  |          | Blue.                                     |
| 30  |          | Yellow.                                   |
| 31  |          | Blue.                                     |
| 32  |          | Orange.                                   |

TABLE II

| I.      | II.                          | III.                                      |
|---------|------------------------------|-------------------------------------------|
| Nr.     | Dyestuff                     | Shade on<br>polyacrylo-<br>nitrile fibres |
| 33..... |                              | Blue.                                     |
| 34..... |                              | Yellow.                                   |
| 35..... |                              | Green.                                    |
| 36..... | C.I. Basic Green 1 (42040)   | Do.                                       |
| 37..... | C.I. Basic Blue 4 (42140)    | Blue.                                     |
| 38..... | C.I. Basic Blue 1 (42025)    | Do.                                       |
| 39..... | C.I. Basic Orange 21 (48036) | Orange.                                   |
| 40..... | C.I. Basic Orange 22 (48040) | Do.                                       |
| 41..... | C.I. Basic Red 13 (48016)    | Pink.                                     |
| 42..... | C.I. Basic Violet 7 (48020)  | Red-violet.                               |
| 43..... | C.I. Basic Yellow 12 (48065) | Yellow.                                   |
| 44..... | C.I. 48013                   | Pink.                                     |
| 45..... | C.I. Basic Blue 6 (61176)    | Blue.                                     |
| 46..... | C.I. Basic Yellow 3 (41006)  | Yellow.                                   |
| 47..... | C.I. Basic Green 4 (42000)   | Green.                                    |
| 48..... | C.I. Basic Red 1 (45160)     | Red.                                      |

We claim:

1. Process for the production of level dyeings on polymeric or copolymeric acrylonitrile fibers, said fibers containing at least 85% acrylonitrile, comprising dyeing this material with an acid dye liquor having a pH in the range between 3.5 to 5 which contains at least one basic dyestuff and a quaternary ammonium compound of the formula



wherein

$R_1$  is an aliphatic hydrocarbon radical of at least eight carbon atoms,

$R_2$  is a lower alkyl radical,

$R_3$  is a lower alkyl radical any substituent of which is selected from hydroxy and phenyl and

$R_4$  is a lower alkylene bridge and

$X^-$  represents the anion of an acid.

2. A process as described in claim 1 wherein  $R_4$  is  $-\text{CH}_2-$ .

3. A process as described in claim 1 wherein  $R_1$  is alkyl of from eight to 14 carbon atoms.

4. A process as described in claim 3 wherein  $R_2$  is methyl or ethyl.

5. A process as described in claim 4 wherein  $R_3$  is selected from methyl, ethyl,  $\beta$ -hydroxyethyl,  $\gamma$ -hydroxypropyl and  $\beta$ -hydroxy- $\beta$ -phenylethyl group.

6. A process as described in claim 1 wherein in the formula of said compound  $R_1$  is alkyl of from eight to 14 carbon atoms, each of  $R_2$  and  $R_3$  represents methyl or ethyl and  $X$  represents chlorine or bromine.

7. A process as described in claim 1 wherein said compound is  $N$ -methyl- $N$ -dodecyl- $N$ - $\beta$ -hydroxy- $\beta$ -phenylethyl- $N$ -2,3-epoxy-propyl-ammonium chloride.

8. A process as described in claim 6, wherein said compound is  $N,N$ -dimethyl- $N$ -dodecyl- $N$ -2,3-epoxypropyl-ammonium chloride.

9. An acid dye liquor for level dyeing on polymeric or copolymeric acrylonitrile fibers containing at least 85% acrylonitrile, which liquor contains at least one basic dyestuff for coloring said fibers, and as a dye assistant a quaternary compound of the formula as described in claim 1.